

# UNITED STATES PATENT OFFICE.

JAMES P. ELLIOTT, OF OAK PARK, ILLINOIS.

## WATERPROOF ROOFING MATERIAL OR THE LIKE AND PROCESS OF MAKING SAME.

1,305,081.

Specification of Letters Patent. Patented May 27, 1919.

No Drawing.

Application filed March 11, 1916. Serial No. 83,559.

To all whom it may concern:

Be it known that I, JAMES P. ELLIOTT, a citizen of the United States, residing at Oak Park, county of Cook, State of Illinois, have invented a certain new and useful Improvement in Waterproof Roofing Materials or the like and Processes of Making Same, and declare the following to be a full, clear, and exact description of the same, such as will 10 enable others skilled in the art to which it pertains to make and use the same.

The material universally employed for making fibrous waterproof sheet roofing material is a low grade felt which, because of its 15 comparative tenacity and capacity for absorbing melted asphalts or tars so as to become saturated with the same, has heretofore encountered no successful competition from other materials, even though the felt, particularly at the present time, is very expensive. Substitutes have been proposed and tried, but they have either lacked tenacity or capacity to absorb the waterproofing materials or have been of such a nature that the 20 cost to manufacture them would be greater than that of the ordinary felt roofing.

My invention has for its object to produce a substitute for felt roofing and the like which shall possess all of the desirable properties of the latter and at the same time be 25 less expensive.

The manufacturer of the roofing usually buys the sheet felt and treats it to render it waterproof and, viewed in one of its aspects, 30 my invention may be said to have for its object to produce a process of making a waterproof fiber substitute for felt roofing and the like which will permit the manufacturer of roofing to employ the same process of finishing raw sheets that he has heretofore employed in waterproofing and finishing felt sheets.

One of the materials that has often been tried as a substitute for the felt is wood pulp 35 which is cheap and possesses sufficient strength; but wood pulp does not readily absorb the usual waterproofing materials and efforts to employ it as a roofing material have therefore been unsuccessful. It has 40 therefore long been recognized that wood pulp is the natural substitute for felt provided it can be waterproofed thoroughly and at not too great a cost. Viewed in one of its aspects my invention may be regarded as 45 having for its object to produce a simple

process of treating wood pulp so as to transform it into a comparatively cheap and efficient waterproof material.

Just as it is desirable to preserve the practices by which the felt is now being treated 60 to render it waterproof, so as not to make it necessary to reorganize or wholly remodel an existing factory, so also is it desirable that there be no interference with the ordinary processes by which wood pulp is produced; 65 and, therefore, viewed in one of its aspects, my invention may be said to have for its object to produce a simple and novel process of manufacturing a waterproofed wood pulp which does not require any change in the 70 process of or machinery for producing ordinary wood pulp.

In accordance with my invention I prepare in dry powdery form a waterproofing material having an asphalt base or, in fact, 75 of any composition which will answer the purpose, and mix this with the wet wood pulp at any suitable stage in the process of manufacturing the latter, preferably in the mixer just before the pulp is rolled out or 80 pressed into sheets. The wood pulp sheets are therefore filled with finely divided, uniformly distributed particles of waterproofing material. These sheets are then treated in exactly the same way as felt is now 85 treated, namely they are immersed in hot waterproofing material which coats the surface and enters into the body of the sheets to a greater or less extent and, because the bath is hot, the fine particles of waterproofing 90 material existing in the sheets are caused to melt and become fluid and thus form an effective seal through which moisture cannot pass.

It will be seen that the addition of the dry 95 powdery waterproofing material to the wood pulp does not interfere with the usual process of making the wood pulp sheets because the operation is exactly the same as if a coloring pigment or other material were added 100 to the pulp in the process of making ordinary pulp. It will also be seen that the process of manufacturing the waterproof material from the wood pulp is the same as that heretofore practised in connection with 105 waterproofing felt. Consequently I have devised a process by means of which it is possible to obtain a very satisfactory substitute for the ordinary waterproofed felt at a cost 110 much less than that of the latter and with-

out making it necessary to disturb existing plants or processes in order to adapt them for the change of material.

It will of course be understood that some 5 of the advantages of my invention or discovery may be obtained by simply subjecting the prepared wood or straw pulp to a sufficient degree of heat to melt the waterproofing material contained therein although the 10 product so produced will of course not be the same as that resulting from the immersion of the prepared wood pulp in a hot bath of waterproofing material.

In order to insure that the particles of 15 waterproofing material contained in the wood pulp shall be liquefied in the hot bath, it is preferable that the dry powdered waterproofing material that is employed be such that it will melt at a lower temperature 20 than that constituting the bath. It is well known to those skilled in the art that the usual waterproofing materials may be made to melt at any desired point within a comparatively wide range of temperatures and 25 therefore no detailed explanation of how this is accomplished is necessary. It will be seen that by having in the pulp a material which will melt at a temperature considerably below that of the bath, very little skill 30 is required to insure that the pulp will remain in the bath long enough to cause the temperature in every portion of the body of pulp to become higher than that at which the waterproofing material will liquefy. 35 It will of course be understood that the main purpose of my invention is to make possible the economical waterproofing of materials that heretofore could not be waterproofed successfully. Some of the advantages 40 of the invention will of course be obtained by using only some of the features thereof. Thus, for example, the powdered waterproofing material may be mixed with the pulp out of which the sheets of felt 45 roofing material are now made; thus greatly shortening the waterproofing process through which the felt must afterward be passed in order to transform it into roofing material. Or, just as in the case of 50 wood or straw pulp, a more or less complete waterproofing may be obtained by simply subjecting the felt made out of the treated pulp to a sufficient degree of heat to melt the contained waterproofing material and 55 cause it to flow.

I claim:

1. The process of manufacturing waterproofed roofing material which consists in mixing with a mass of pulp small particles 60 of waterproofing material, working the pulp into the form of a sheet in the usual way, and then subjecting the sheet to a hot bath of liquefied waterproofing material in the manner in which ordinary felt roofing is 65 commonly treated to waterproof it.

2. The method of producing waterproof sheet roofing which consists in incorporating in the sheet small particles of waterproofing material and then immersing the sheet in the usual way in hot liquefied waterproofing material. 70

3. The process of producing a waterproofed sheet roofing material which consists in making a sheet out of pulp in the usual way with the addition of small particles of waterproofing material to the pulp at any convenient point in the process of making the sheet, and then immersing the sheet in a hot liquefied waterproofing bath in the manner now employed for waterproofing ordinary felt roofing material. 80

4. The process of producing a waterproofed body or sheet which consists in making it of pulp having small particles of waterproofing material distributed throughout the mass thereof, and then immersing it in a hot bath of liquid waterproofing material. 85

5. The process of producing a waterproofed body or sheet which consists in 90 making it of pulp having small particles of waterproofing material distributed throughout the mass of the same, and then subjecting it to a hot bath of liquefied waterproofing material whose melting point is higher 95 than that of the first-mentioned waterproofing material.

6. The process of producing fibrous waterproof sheet roofing material which consists in forming a sheet out of pulp in 100 the usual way and, in the process of formation of the sheet without the addition of heat, adding finely divided waterproofing material to the pulp; and then immersing the sheet in a hot bath to melt the waterproofing material. 105

7. The process of producing fibrous waterproof sheet roofing material which consists in forming a sheet out of pulp in the usual way and, in the process of formation of the sheet without the addition of heat, adding finely divided waterproofing material to the pulp; and then simultaneously applying heat and liquid waterproofing material to the sheet to melt the waterproofing material in the sheet and at the same time produce a waterproof coating on the exterior of the sheet. 115

8. The process of producing a waterproofed body or sheet which consists in 120 making it of pulp having small particles of waterproofing material distributed throughout the mass of the same, and then subjecting it to a hot bath of liquefied waterproofing material whose temperature is higher 125 than the melting point of the first mentioned waterproofing material.

9. The process of producing a waterproofed body or sheet which consists in intimately mixing wet pulp with finely-divided 130

- asphalt, working the wet mixture into the desired shape, and then subjecting it to a hot bath of liquefied waterproofing material whose temperature is higher than the melting point of the said asphalt. 5
10. The process of producing a waterproofed body or sheet which consists in intimately mixing wet pulp with finely-divided asphalt, working the wet mixture into the desired shape, and then subjecting it to a hot bath containing asphalt and having a temperature higher than the melting point of the first mentioned asphalt. 10
11. The process of producing fibrous waterproof sheet roofing material which consists in forming a sheet out of pulp in the usual way and, in the process of formation of the sheet without the addition of heat, adding finely-divided asphalt to the pulp; and then immersing the sheet in a hot bath to melt the asphalt. 15
12. The process of producing a waterproofed body or sheet which consists in intimately mixing wet pulp and finely-divided asphalt, shaping the wet pulp while the asphalt still remains in its finely-divided state and without changing it from such finely-divided state, and then simultaneously coating the body or sheet and melting the asphalt content thereof. 20
13. As an article of manufacture, a sheet of flexible and porous unsaturated building felt consisting of waterproofing material in comminuted form and other material. 25
14. As an article of manufacture, a sheet of flexible and porous unsaturated building felt consisting of fusible waterproof material in comminuted form and other material. 30
15. As an article of manufacture, a sheet of flexible and porous unsaturated building felt comprising a waterproofing material in comminuted form and paper stock material. 35
16. As an article of manufacture, a sheet of flexible and porous unsaturated building felt comprising asphalt in comminuted form and a fibrous material. 40
17. As an article of manufacture, a sheet of flexible and porous unsaturated building felt consisting of fusible waterproofing material in comminuted form and a fibrous material. 45
18. The process of producing fibrous waterproof sheet building felt which consists in forming a flexible porous sheet out of comminuted fusible waterproofing material mixed with a fibrous material, and then applying heat to the sheet in order to melt the waterproofing material. 50
19. The process of producing fibrous waterproof sheet building felt which consists in forming a flexible porous sheet out of comminuted asphalt mixed with a fibrous material, and then applying heat to the sheet in order to melt the asphalt. 55

In testimony whereof, I sign this specification. 60

JAMES P. ELLIOTT.